

## 1

2,938,815

### PROCESS FOR MAKING CELLULOSE MATERIALS ROTPROOF

Cornelis van Bochove, The Hague, and Hendrik J. Hueck, Delfgauw, Netherlands, assignors to Nederlandse Organisatie voor Toegepast-Natuurwetenschappelijk Onderzoek ten behoeve van Nijverheid, Handel en Verkeer, The Hague, Netherlands

No Drawing. Filed June 30, 1958, Ser. No. 745,326

Claims priority, application Netherlands July 4, 1957

5 Claims. (Cl. 117—138.5)

It has been found that cellulose materials such as cotton can be protected against rotting by treating them with chloracetamide and formaldehyde in a molar ratio of 1 mol chloracetamide on not more than 1 mol formaldehyde; instead of this the material can also be treated with methyolchloracetamide.

The effect is specific; only instead of chloracetamide, bromacetamide or iodoacetamide may be used, but for practical purposes this is unnecessarily expensive. With other halogen carboxylic acid amides one does not nearly obtain the same effect as with chloracetamide. The same holds good for the unsubstituted acid amides. The methyol compounds of the following materials have been examined for example:

Acetamide  
Butyramide  
Capronamide  
Beta-chloropropionamide  
Dichloracetamide

35 but the effect found, if any, was negligible. Neither did a treatment with formaldehyde only, yield a rotproof product.

As it is sufficient for the reaction when one mol of formaldehyde is present per mol of chloracetamide, and an excess of formaldehyde therefore not only means a waste but may moreover be detrimental not more than one mol of formaldehyde should be present per mol of halogen acetamide. By formaldehyde is also meant a material yielding formaldehyde such as paraldehyde.

The invention will be illustrated with regard to the treatment of cotton; the protection of cotton against rotting is namely very important and therefore this treatment has been subjected to the most detailed examination.

The particulars given below are obtained with the following materials:

Standard fabric of 100% cotton;  
Weight per m.<sup>2</sup>: 270 gr.;  
Number of threads per 10 cm.: warp 334; woof 198;  
Yarn English: warp 31, 3/2 (18.9x2); woof 21, 2/2 (27.9x2).

In impregnating a foulard was used:

Fabric speed: 0.7 m./min.;  
Squeezing pressure: 350 kg. across 28 cm. fabric width;  
Squeezing yield: about 60%.

## 2

The drying and after-heating took place under the following circumstances:

Drying temperature: 70° C.;

Drying time: 10 min.;

5 Temperature during after-treatment: see below;  
Time: 4½ min.

In order entirely to remove material which might not have reacted, the foulard was rinsed a few times with 10 cold water first, and afterwards twice with water of 70° C.

The burying tests and the tensile strengths were determined according to instruction Vitno-Bio Al.

15 The treatment is carried out as follows by way of example.

The cotton was impregnated with a solution of methyolchloracetamide in water to which a catalyst was added (e.g. oxalic acid). After drying a treatment at a higher temperature (130°—140°) followed which lasted a few 20 minutes, and during which the reaction proper took place. After this rinsing was effected.

The cotton treated in this way was subjected to a burying test. After 1, 2 and 4 weeks a number of strips was removed and the tensile strength determined. As a 25 criterion for the behaviour in the ground the rest strength was taken. The definition of "rest strength" is as follows: the ratio between the tensile strengths after and before the burying, expressed in percents.

The results of a number of these experiments was as 30 follows:

Table 1.—Results of burying tests of cotton, treated with methyolchloracetamide

| Test No.    | Degree of substitution <sup>1</sup> | blank tensile strength (kg./25 mm.) | rest strength (percent) after— |         |         |
|-------------|-------------------------------------|-------------------------------------|--------------------------------|---------|---------|
|             |                                     |                                     | 1 week                         | 2 weeks | 4 weeks |
| R 31-40     | 0.5                                 | 46                                  | 61                             | 7       | 0       |
| R 31-41     | 1.2                                 | 39                                  | 92                             | 56      | 36      |
| R 31-42     | 2.2                                 | 38                                  | 105                            | 61      | 32      |
| Z 2-17      | 3.1                                 | 39                                  | 85                             | 67      | 41      |
| Z 2-18      | 4.2                                 | 37                                  | 95                             | 92      | 62      |
| Z 2-19      | 5.8                                 | 35                                  | 94                             | 100     | 83      |
| R 31-53     | 5.9                                 | 26                                  | 100                            | 85      | 92      |
| not treated |                                     | 44                                  | ca. 10                         | 0       | 0       |

<sup>1</sup> Expressed in the number of side groups per 100 glucose units.

From these results it can be concluded that there is an evident correlation between the degree of substitution and the resistance against the influence of micro-organisms. Complete resistance for four weeks of burial is obtained at a substitution degree of about 6. When one week of burial is chosen as a criterion, a substitution degree of 1 to 2 is sufficient. These degrees of substitution are extraordinarily low, as compared to other 55 methods for making cellulose material rotproof by chemical modification, such as acetylating and cyanoethylating, in which at least ½ of the total number of OH-groups of the cellulose should be replaced to ensure success, which, however, implies a drastic change of the qualities. The effect at the above-mentioned very low degrees of substitution is strictly specific of the process according to the invention.

60 Besides a burying test a few samples of treated cotton were subjected to a treatment with enzyme solution for 65 two weeks.

The results of this can be summarized as follows:

Table 2.—Cotton treated with methylolchloracetamide

| Test No.    | Degree of substitution | influence of enzyme treatment       |                                               |                                              |
|-------------|------------------------|-------------------------------------|-----------------------------------------------|----------------------------------------------|
|             |                        | blank tensile strength (kg./25 mm.) | rest strength after enzyme treatment, percent | rest strength after 1 week's burial, percent |
| not treated |                        | 44                                  | 44                                            | 0-40                                         |
| R 31-40     | 0.5                    | 44                                  | 63                                            | 61                                           |
| R 31-41     | 1.2                    | 36                                  | 89                                            | 92                                           |
| R 31-42     | 2.2                    | 39                                  | 89                                            | 105                                          |
| R 31-53     | 5.9                    | 26                                  | 96                                            | 100                                          |

For purposes of comparison the results after 1 week's burial have been inserted in this table.

In this test too it appeared, that the cotton is made resistant by the reaction with methylolchloracetamide. The results of this test correspond more or less to those of 1 week's burial.

As a matter of course one is neither bound to the above-mentioned specifications of the fabric, nor to the details of impregnating, drying and after-treatment.

In order to obtain more certainty about the effect of the bonded chloracetamide, examination was made, as to what influence "loosely" applied chloracetamide had on the resistance of cotton. To this end cotton was impregnated with solutions of chloracetamide and methylolchloracetamide respectively in water. Both compounds were applied to the fabric in various concentrations, which corresponded more or less to the quantity of "bonded" chloracetamide.

The impregnated fabrics were subjected to a burying test. Results:

Table 3.—Comparison of "bonded" and "loose" methylolchloracetamide

| Test No. | Treatment                        | Number of molecules chloracetamide per 100 glucose units | rest strength |         |         |
|----------|----------------------------------|----------------------------------------------------------|---------------|---------|---------|
|          |                                  |                                                          | 1 week        | 2 weeks | 4 weeks |
| R 31-58  | chloracetamide (loose).          | 4.2                                                      | 31            | 2       | 0       |
| R 31-59  |                                  | 4.6                                                      | 33            | 2       | 0       |
| R 31-60  |                                  | 7.3                                                      | 63            | 2       | 0       |
| R 31-50  | methylolchloracetamide (loose).  | 3.0                                                      | 52            | 1       | 0       |
| R 31-51  |                                  | 5.4                                                      | 96            | 30      | 0       |
| R 31-42  | methylolchloracetamide (bonded). | 2.2                                                      | 105           | 61      | 32      |
| R 31-53  |                                  | 5.9                                                      | 100           | 85      | 92      |

It is clear that "loose" chloracetamide has hardly any effect at all.

The influence of the variables in the process according to the invention was further examined.

During the reaction of cellulose with methylolchloracetamide the following variables occur:

(1) Concentration of methylolchloracetamide in the impregnating liquid;

(2) Nature and quantity of the catalyst used.

(3) Temperature and duration of the after-heating.

In this reaction the quantity of bonded chloracetamide is a criterion for the degree of conversion. Besides that, this kind of reactions requires that the mechanical properties of the cotton may not be subject to any or scarcely to any alterations. A criterion for this is the tensile strength.

Investigation was now made as to what influence some of the above-mentioned variables had on the attained degree of substitution and on the loss of tensile strength.

(1) Influence of the concentration of the methylolchloracetamide.

A series of tests was carried out, in which a cotton was

impregnated with solutions of methylolchloracetamide in water with a content varying from 2 to 20%.

The results are given in Table 4.

Table 4.—Connection between bath concentration and degree of substitution and tensile strength

Reaction conditions:

pH of the impregnating bath: 2.5

Catalyst: oxalic acid

Drying at 70°-80° C.

After-heating: 5 min. at 140° C.

15

| Test No. | Methylolchloracetamide (percent) | Degree of substitution, percent | Tensile strength (kg./25 mm.) | Loss of tensile strength, percent |
|----------|----------------------------------|---------------------------------|-------------------------------|-----------------------------------|
| R 31-40  | 2                                | 0.5                             | 46                            | -----                             |
| R 31-41  | 5                                | 1.2                             | 39                            | 11                                |
| R 31-42  | 10                               | 2.2                             | 38                            | 14                                |
| Z 2-17   | 13.3                             | 3.1                             | 39                            | 11                                |
| Z 2-18   | 16.7                             | 4.2                             | 37                            | 16                                |
| Z 2-19   | 20.0                             | 5.8                             | 35                            | 20                                |

(2) Influence of nature and quantity of the catalyst used and of the temperature of after-heating. Oxalic acid was chosen for a catalyst.

25

With oxalic acid as a catalyst the pH was adjusted to 4.5 and 2.5. Besides this a test was carried out with a pH of 6.5, which was obtained by adding a few drops of NaOH to a solution of methylolchloracetamide, which in itself had a pH of about 5.5. So here no oxalic acid was added.

The results are given in Table 5.

Table 5.—Influence of the pH of the impregnating bath and the reaction temperature on the degree of substitution

35 Reaction conditions:

Bath concentration 16.7%,

After-heating at 130°, 140° and 150° C. respectively for 5 minutes.

40

| Test No.   | pH  | Temperature (° C.) | Degree of substitution, percent | Loss of tensile strength, percent |
|------------|-----|--------------------|---------------------------------|-----------------------------------|
| Z 2-26-1 a | 6.5 | 130                | 0.5                             | 4                                 |
|            |     | 140                | 3.0                             | 10                                |
|            |     | 150                | 2.8                             | 29                                |
| Z 2-26-2 a | 4.5 | 130                | 0.7                             | 6                                 |
|            |     | 140                | 1.6                             | 8                                 |
|            |     | 150                | 5.5                             | 40                                |
| Z 2-26-3 a | 2.5 | 130                | 0.7                             | 0                                 |
|            |     | 140                | 4.2                             | 10                                |
|            |     | 150                | 7.8                             | 60                                |

From all these tests it is evident, that by the treatment according to the invention a product is obtained which is extremely rotproof.

55

Some tests were carried out in order to compare the present process with known processes.

(1) Influence of repeated washing and dry-cleaning on the rotproofness of cotton, treated in the following ways:

60

- According to the invention (substitution degree 6; cf. Table I);
- Copper naphthenate (approx. 0.7% Cu);
- Lauryl-pentachlorophenol (+water repellent agent) (approx. 2%).

65

These three samples were washed 5 times and dry-cleaned 5 times. Both treatments were carried out in a conventional domestic washing machine manufactured by the Allgemeine Elektrizitäts Gesellschaft, a well known manufacturing firm of West Germany.

For the washing the washing agent "Savonine Compleet" was used. Savonine Compleet stands for a detergent of the following composition in percent by weight: common soap 20%; sodium carbonate anhydrous 45%; sodium meta silicate 9H<sub>2</sub>O 12%; sodium salt of carboxy methyl cellulose (NaCMC) 1.2%; the rest wa-

ter. This preparation was applied in a quantity of 10 g./litre. The weight ratio of dry sample to bath liquid was 1:20. The washing took place for one quarter of an hour at 80° C. After this rinsing in distilled water took place twice, each time for 5 minutes, and drying at 60° C.

Dry-cleaning took place in trichloroethylene at 20° C. for 10 minutes. After this drying at the air took place.

After the termination of the washing tests the samples were subjected to a burying test for two and four weeks.

In Table 6 below is indicated what precentual rest strengths the strips had that had been buried.

Table 6

| Sample                     | After 2 weeks' burial |                 |                      | After 4 weeks' burial |                 |                      |
|----------------------------|-----------------------|-----------------|----------------------|-----------------------|-----------------|----------------------|
|                            | immediately           | 5 times washing | 5 times dry cleaning | immediately           | 5 times washing | 5 times dry cleaning |
| according to the invention | 93                    | 84              | 98                   | 85                    | 73              | 84                   |
| copper naphthenate         | 98                    | 83              | 96                   | 99                    | 44              | 81                   |
| lauryl-pentachlorophenol   | 100                   | 0               | 0                    | 48                    | 0               | 0                    |
| not treated                | 0                     | 0               | 0                    | 0                     | 0               | 0                    |

From this the following is apparent:

Washing and dry-cleaning have only very little influence on the rotproofness of cotton which has been treated according to the invention.

Cotton treated with copper naphthenate will stand dry-cleaning, but does not stand washing quite as well.

The effect of lauryl-pentachlorophenol disappears entirely, both by dry-cleaning and by washing.

These results clearly show the difference between the effect of chemical reaction with the cellulose according to the invention and the effect of impregnating "loosely" with the usual fungicides.

Some exposition tests were also carried out.

On the roof of a building a comparative test was carried out in a number of racks, in which a number of cotton strips, which had been treated in various ways, were exposed to the sunlight. In this test one half of the strips was put behind frames of Plexiglas, by which the influence of the sunlight was not eliminated, but that of the rain was.

After the termination of the exposition (1, 2, 4 and 8 months) a certain number of the strips were subjected to a burying test (2 weeks).

The following treatments were applied:

- (a) Treatment according to the invention (degree of substitution 6);
- (b) Treatment with copper naphthenate (0.8% Cu);
- (c) Treatment with lauryl-pentachlorophenol + water repellent agent;
- (d) Treatment with copper-8-oxyquinoline (0.7% Cu).

In the following Table 7 the rest strengths (in percents of the non-buried samples) are again given.

Table 7

| 5  | Sample: original         | exposed           |    |    |    |                 |    |    |    |
|----|--------------------------|-------------------|----|----|----|-----------------|----|----|----|
|    |                          | uncovered, months |    |    |    | covered, months |    |    |    |
|    |                          | 1                 | 2  | 4  | 8  | 1               | 2  | 4  | 8  |
| 10 | not treated              | 0                 | 0  | 14 | 18 | 2               | 0  | 3  | 7  |
| 15 | acc. to the invention    | 89                | 81 | 98 | 63 | 38              | 86 | 85 | 84 |
| 15 | Cu-naphthenate           | 97                | 96 | 98 | 25 | 4               | 93 | 89 | 83 |
| 15 | lauryl-pentachlorophenol | 97                | 20 | 21 | 11 | 6               | 48 | 37 | 32 |
| 15 | Cu-8-oxyquinoline        | 100               | 69 | 18 | 15 | 3               | 94 | 94 | 92 |

From these results it is evident that cotton treated according to the invention, when exposed to atmospheric influences, is much slower to lose its rot-preventing qualities than cotton which has been impregnated according to the usual processes. This should be ascribed to the chemical reaction which has taken place when treating it with methylolchloracetamide.

What we claim is:

1. Process for improving the resistance against micro-biological attack of cellulose-containing materials by impregnating the material with an aqueous solution of halogeno-acetamide and formaldehyde and an acid catalyst, the amount of formaldehyde being not greater than one mole per mole of halogeno-acetamide, drying the impregnated material and subjecting it to a temperature of between 110 and 160° C.
2. The process of claim 1 wherein the acid catalyst is oxalic acid.
3. Process for improving the resistance against micro-biological attack of cellulose-containing materials by impregnating the material with an aqueous solution of a methylol-halogeno-acetamide and an acid catalyst, drying the impregnated material and subjecting it to a temperature of between 110 and 160° C.
4. The process of claim 3 wherein the treating agent is methylol chloroacetamide.
5. The process of claim 3 wherein the acid catalyst is oxalic acid.

#### References Cited in the file of this patent

#### UNITED STATES PATENTS

- 2,270,520 Riehen ----- Jan. 20, 1942  
 2,446,864 Abrams ----- Aug. 10, 1948  
 2,587,957 Bauer et al. ----- Mar. 4, 1952

#### FOREIGN PATENTS

- 495,714 Great Britain ----- Nov. 14, 1938